

## 1

3,369,893

### COPPER-ZINC ALLOYS

William R. Opie, Keyport, N.J., and Jan A. Paces, New York, N.Y., assignors to American Metal Climax, Inc., New York, N.Y., a corporation of New York  
No Drawing. Filed Dec. 28, 1964, Ser. No. 421,668  
6 Claims. (Cl. 75—157.5)

The present invention relates to alloys and, more particularly, to copper-zinc alloys in which copper is the predominant ingredient.

It is well known that copper-zinc alloys, commonly called "brasses" and under certain circumstances "bronzes," are of considerable engineering and commercial importance and are widely employed in both cast and fabricated conditions. These alloys would of course assume even greater importance if their physical or mechanical properties and/or characteristics could be improved. For example, an increase in tensile strength would permit the use of such alloys in a much wider variety of structural applications. However, oftentimes an increase in tensile strength is accompanied by a decrease in another important property or characteristic, e.g., ductility, corrosion resistance, fabricability, impact strength, electrical or thermal conductivity, etc. Thus, the art has been faced with the difficult problem of increasing the tensile strength of copper-zinc alloys without unduly or detrimentally decreasing another valuable property and/or characteristic. The solution of this problem is rendered even more difficult by the usual requirement that the strengthened yet ductile alloy be economically producible.

Still other problems arise in connection with the economic production of high-strength copper-zinc alloys. One of these further problems is related to the metallurgical properties and characteristics of these copper-containing alloys. For example, wrought copper alloys including the copper-zinc alloys are often subjected to a stress-relieving or annealing heat treatment. After such a stress-relieving treatment, the tensile strengths of the copper-containing alloys usually fall off considerably and disadvantageously. Accordingly, what is needed is a copper-zinc alloy that retains much of its tensile strength even after stress-relieving or annealing.

Another problem concerns modern day technological demands for copper-zinc alloys having good high temperature properties and characteristics as well as the other aforementioned properties, characteristics and advantages. This problem is somewhat related to the problem of producing copper-zinc alloys having high tensile strengths in the stress-relieved condition. Consequently, those alloys having the higher strengths in the stress-relieved state are ordinarily the alloys having the better tensile strengths at high temperatures.

The art has attacked these myriad problems in a number of ways. For example, in order to obtain the higher strength copper-zinc alloys, the art has in many cases turned to the addition of alloying element or elements thereto. Such elements may retain their elemental identity or enter into solid solution or form special constituents depending upon the specific amounts present and the remaining ingredients of the alloy. How it is hardened may be important since the properties and characteristics, particularly at high temperature, may be dependent on the strengthening means. Consequently, the proper strengthening means presents a new problem.

Although many attempts were made to overcome the

## 2

foregoing difficulties and other disadvantages, none, as far as we are aware, was entirely successful when carried into practice commercially on an industrial scale.

It has now been discovered that copper-zinc alloys having high strength and other advantageous properties and/or characteristics together with ductility may now be economically produced.

It is an object of the present invention to provide new copper-zinc alloys having a unique combination of properties and/or characteristics.

Another object of the present invention is to provide novel copper-zinc alloys which have beneficial properties and/or characteristics in the stress-relieved condition.

The invention also contemplates providing new copper-zinc alloys having excellent strength in the wrought condition.

It is a further object of the invention to provide novel copper-zinc alloys that are readily fabricatable.

Still another object of the instant invention contemplates new copper-zinc alloys having high strength in combination with adequate ductility.

One of the other objects of this invention is to provide novel high-strength copper-zinc alloys having good thermal and electrical conductivity.

A further object of the invention contemplates the provision of copper-zinc alloys having a unique combination of ingredients in special proportions.

Among the further objects of the present invention is the provision of a special economic process for hardening copper-zinc alloys.

Other objects and advantages will become apparent from the following description:

Generally speaking, the present invention contemplates the production of unique copper-base alloys which have high strength and adequate ductility even when stress-relieved or annealed at temperatures as high as 350° C. or higher. The alloys of this invention contain, in weight percentages, about 0.05% to about 0.35%, e.g., about 0.1%, beryllium, about 0.08% to about 0.5%, e.g., about 0.2%, titanium, up to about 0.5% chromium, up to about 10% aluminum, e.g., about 7%, and from about 10% to about 45% zinc with the sum of the aluminum and zinc percentages lying between about 10% and 45%. The remaining ingredient of these alloys apart from incidental elements, including impurities and residual deoxidizers, is copper in amounts of at least about 54.5%. The alloys of this invention containing the aforementioned ingredients in the aforementioned proportioned amounts are characterized by a high recrystallization temperature, refined grain structure and resistance to grain growth at elevated temperatures, e.g., 300° C., 500° C. or even higher.

Another unique feature of the alloys within the scope of the present invention is that high strengths are obtained without any detrimental decrease in electrical and/or thermal conductivity.

The alloys according to this invention contain copper, zinc, titanium and beryllium in specially controlled amounts and each of these elements in combination with each other element plays an important part in controlling the properties and/or characteristics of the alloy. For example, the beryllium content is in the range of about 0.05% to about 0.35%, e.g., about 0.1%, and, advantageously, between about 0.05% and 0.085% by weight of the alloy. The inclusion of beryllium in the amounts specified in the copper-zinc alloys of this invention aids

in improving the tensile strength when appropriate amounts of titanium are copresent. Furthermore, the beryllium inclusion in combination with the remaining ingredients beneficially raises the recrystallization temperature and permits the alloy to be employed in high temperature applications. Thus, with the higher recrystallization temperature, by grain growth is retarded and the alloy remains stronger at the more elevated temperatures, e.g., 500° C., than when beryllium is not present. In addition to its other functions, the beryllium may act as a deoxidizer. When used as a deoxidizer, enough beryllium should be employed to assure that the copper-zinc alloy contain beryllium in the amounts hereinbefore set forth. However, if too much beryllium is used (more than about 0.35%), the ductility of the resulting alloy is very low and is quite difficult to work. Furthermore, the inclusion of beryllium in amounts above 0.35% may be undesirable if cost is an important factor. For optimum strength and workability in combination with low cost, the maximum amount of beryllium is about 0.085%. If too little beryllium is used, e.g., less than about 0.05%, the strengths of the copper-zinc alloys suffer.

It was found that titanium, when used in the amounts hereinbefore set forth in combination with the beryllium in the copper-zinc alloys of this invention, has an effect similar to that of beryllium. For example, the titanium (together with beryllium) aids in the strengthening or hardening of copper-zinc alloys. However, the combined use of beryllium and titanium yields an even stronger alloy than is expected. Like beryllium, if too much is used, e.g. more than about 0.5% by weight of the alloy, the ductility and fabricability detrimentally decreases and if too little is used, e.g. less than about 0.08% the strength detrimentally decreases. Also like beryllium, the titanium may have a deoxidizing effect when desired. In this situation, it is important that enough titanium be employed to insure that the copper-zinc alloy contains quantities of titanium within the range hereinbefore set forth. Titanium also has at least two other important functions. Firstly, titanium substantially inhibits zinc-fuming, i.e., the volatilization of zinc. Secondly, titanium apparently prevents the copper-zinc alloys containing beryllium from somewhat losing a portion of their strength at the more elevated temperatures, e.g., 300° C. Advantageously, the titanium content is between about 0.08% to about 0.12% by weight of the alloy for optimum properties and characteristics.

The zinc content should be kept within the specified range of from 10 to 45% in order to provide the desired results. If the zinc content is too high, the ductility is appreciably and undesirably reduced. If the zinc content is below about 10%, the strength of the copper-zinc alloys of this invention are adversely affected. Part of the zinc may be replaced by aluminum when still higher strengths or greater oxidation resistance is desired. However, as is known, these higher strengths and oxidation resistance are achieved at the expense of castability, workability and conductivity. In this connection, the alloy may contain up to about 10% aluminum which replaces zinc in an amount equal to the amount of aluminum added. However, the alloys of this invention must always contain at least about 10% zinc and the sum of the aluminum and zinc percentages does not exceed about 45%. Advantageously, particularly where the soldering of the alloys is an important factor, the aluminum content is up to about 5% since aluminum, particularly in the higher end of the range, tends to form an oxide film which is detrimental during the fluxing phase of the soldering process.

The copper-zinc alloys of this invention containing controlled amounts of beryllium and titanium may include up to 0.5%, e.g., up to about 0.1%, chromium by weight of the alloy. Advantageously, the alloy does contain chromium in amounts of between 0.015% and 0.02% since chromium contributes to the strength of the alloy while

affording some increase in the corrosion resistance of the alloys of this invention.

The alloys of this invention may also contain incidental elements such as up to about 0.5% silicon, up to about 1.5% iron, up to about 0.05% phosphorous, up to about 0.5% magnesium, up to about 1% tin, up to about 0.5% zirconium, up to about 2% manganese, up to about 0.5% lead, up to about 1% nickel and up to about 1% cobalt provided that the sum of such incidental elements is below about 3%, e.g. 1%. In this connection, when the alloys of this invention contain one or more of the aforementioned incidental elements, the amounts present are at the expense of the zinc content on a weight-per-weight basis. However, even when such element or elements are present, the minimum zinc is still at least about 10% by weight of the alloy. Accordingly, the sum of zinc, aluminum and incidental ingredients is between about 10% and about 45%.

Advantageously, the incidental elements are kept below their solubility limits in the copper-zinc alloys of this invention. In particular, tin should be kept below about 1% by weight of the alloy since it has a tendency to form a phase having the appearance of the brittle delta phase of the copper-tin series. However, its inclusion in amounts of less than about 1% may afford some additional resistance to oxidation. Iron, while its inclusion may be desirable as a grain refiner, should be kept below about 1.5% since the iron-rich constituent is preferentially attacked in corrosive media. As is well known, lead is included to improve machinability but it seriously weakens the alloy and its inclusion in the alloys of this invention should be minimized. Nevertheless, the fact that the alloys of this invention can tolerate up to about 0.5% lead, e.g., up to about 0.25%, is a quite important practical advantage since it permits the use of scrap in melting the alloy. Manganese additions increase the amount of any iron present that may go into solution. In addition, it can be present in greater amounts, e.g., about 3% with the higher aluminum contents, e.g., from about 5% to about 10%, since it appears to extend the range of ductile copper-zinc alloys containing aluminum. The alloys of this invention may also tolerate up to about 0.1% lithium although care should be taken to see that the uppermost portion of the range is not exceeded since lithium adversely affects workability and fabricability. Advantageously, each of the aforementioned incidental elements is kept below about 0.3% in order to achieve optimum properties and characteristics in the alloy and below about 0.1% where conductivity is an important factor.

In carrying the invention into practice, particularly unexpected results are obtained when the alloys contain, in weight percentages, about 0.05% to about 0.085% beryllium, about 0.08% to about 0.12% titanium, about 0.015% to about 0.02% chromium, up to about 5% aluminum, about 15% to about 40% zinc with the sum of the aluminum and zinc percentages being about 15% to about 40% and the balance, apart from incidental elements including magnesium, lead, tin, iron, zirconium, nickel and manganese in amounts up to about 1.5% in all, being copper in amounts of at least about 60%. Such alloys have a superior combination of physical, mechanical and/or metallurgical properties and/or characteristics. For example, the alloys have a transverse ultimate tensile strength (U.T.S.) of at least about 100,000 pounds per square inch (p.s.i.) in the 60% cold-worked condition and a transverse U.T.S. of at least about 50,000 p.s.i. after stress-relieving at about 450° C. for about one hour.

For the purpose of giving those skilled in the art a better understanding of the invention and a better appreciation of the advantages of the invention the following examples are set forth. In these examples, a series of castings having varying copper and zinc contents were prepared. Charges of copper were melted and the other alloying constituents were added to the respective charges as master alloys, e.g., copper-titanium, copper-beryllium

and copper-chromium. However, as those skilled in the art will readily appreciate, the alloying additions may be plunged into the melt in their element state. Finally, zinc was added to the melt and the alloys were cast into a graphite mold at 1050° C. The compositions of these alloys in weight percentages are set forth in Table I.

TABLE I

| Alloy    | Copper (percent) | Zinc (percent) | Beryllium (percent) | Titanium (percent) | Chromium (percent) |
|----------|------------------|----------------|---------------------|--------------------|--------------------|
| A* ----- | 69.8             | 30             | 0.081               | 0.12               | 0.016              |
| B-----   | 59.8             | 40             | 0.08                | 0.11               | 0.019              |
| C-----   | 79.7             | 20             | 0.073               | 0.11               | -----              |
| D-----   | 89.6             | 10             | 0.071               | 0.11               | 0.016              |

\*Also contained 0.021 magnesium (incidental element).

The resulting slabs were scalped, preheated at about 600° C. for about 30 minutes and hot worked to an intermediate thickness of about 0.1". After stress-relieving or annealing at about 450° C. for about one hour, the alloys were cold rolled to spring hardness, i.e., 60% reduction.

Table II lists the results of mechanical testing after about 60% cold work (spring hard) and after stress-relieving at various temperatures for various times in hours (hrs.). In addition, Table II includes testing to determine the conductivity in relation to the International Annealed Copper Standard (I.A.C.S.).

TABLE II

| Alloy  | Condition               | Transverse U.T.S. (p.s.i.) | Transverse Elongation (percent) | Hardness (Rockwell B) | Conductivity (percent I.A.C.S.) |
|--------|-------------------------|----------------------------|---------------------------------|-----------------------|---------------------------------|
| A----- | Spring Hard (SH)-----   | 131,000                    | 3                               | 97                    | 26                              |
| A----- | SH+340° C., 4 hrs.----- | 129,000                    | 1                               | 100                   | 26                              |
| A----- | SH+450° C., 1 hr.-----  | 120,000                    | 5                               | 93                    | 27                              |
| A----- | SH+500° C., 1 hr.-----  | 83,000                     | 20                              | 80                    | 27                              |
| A----- | SH+550° C., 1 hr.-----  | 74,000                     | 25                              | 73                    | 27                              |
| B----- | SH-----                 | 137,000                    | 3                               | 98                    | 30.5                            |
| B----- | SH+340° C., 4 hrs.----- | 92,000                     | 20                              | -----                 | 30                              |
| B----- | SH+450° C., 1 hr.-----  | 84,000                     | 28                              | 70                    | 28                              |
| B----- | SH+550° C., 1 hr.-----  | 76,000                     | 30                              | -----                 | 28                              |
| C----- | SH-----                 | 140,000                    | 3                               | 96                    | 30                              |
| C----- | SH+340° C., 4 hrs.----- | 110,000                    | 3                               | -----                 | 30                              |
| C----- | SH+450° C., 1 hr.-----  | 61,000                     | 36                              | 93                    | 31                              |
| C----- | SH+550° C., 1 hr.-----  | 55,000                     | 44                              | -----                 | 31                              |
| D----- | SH-----                 | 107,000                    | 2                               | 84                    | 30.5                            |
| D----- | SH+450° C., 1 hr.-----  | 97,500                     | 5                               | 79                    | 34                              |

By comparison, the corresponding properties obtained with a conventional 70:30 brass nominally containing, by weight, about 70% copper, about 30% zinc and less than 0.05% incidental elements, including impurities, when subjected to the same treatment as applied to alloys A, B, C and D, are shown in Table III.

TABLE III

| Condition               | Transverse U.T.S. (p.s.i.) | Transverse Elongation (percent) | Hardness (Rockwell B) | Conductivity (percent I.A.C.S.) |
|-------------------------|----------------------------|---------------------------------|-----------------------|---------------------------------|
| Spring Hard-----        | 103,000                    | 2                               | 95                    | 26                              |
| SH+340° C., 4 hrs.----- | 60,000                     | 40                              | 51                    | 28                              |
| SH+450° C., 1 hr.-----  | 56,000                     | 44                              | -----                 | 28                              |

When stress-relieved at 550° C. for about one hour, the conventional 70:30 brass was dead soft.

By comparing alloy A with the conventional 70:30 brass of Table III, it is clear that the alloys of the invention have much the superior tensile properties particularly after stress-relieving thus indicating the high temperature utility of the alloys of the present invention. As a matter of fact, alloy A (within the scope of the invention and containing amounts of copper and zinc comparable with the amounts contained in the conventional brass) exhibited over a 100% higher transverse tensile strength after being stress-relieved at 450° C. over

that of the conventional brass subjected to identical treatment. In other words, the strength of the conventional brass was more than doubled by additions of controlled amounts of beryllium and titanium. Furthermore, the conductivity of the higher strength copper-zinc alloys of this invention is similar to that of the conventional 70:30 brass.

The alloys of the present invention, by virtue of their high strength even after a relatively high-temperature stress-relief, permit a greater use to be made of copper-zinc alloys in more severe structural applications, including high temperature applications. In view of these properties and/or characteristics, the alloys of the present invention can be used in high pressure radiators and other high strength applications necessitating the use of solder. In this connection, it is important to bear in mind that the resistance to softening of the alloys during stress-relieving at elevated temperature permits the use of cheaper and stronger solders over those previously used (which contain too much tin) to join the copper-zinc alloys to similar or dissimilar metals. Moreover, their use in electrical applications is not in any manner restricted particularly when compared with the conventional 70:30 brass since the conductivity of the alloys of the present invention is similar to the aforementioned conventional brasses. Furthermore, the uses for the alloys is greatly

enhanced by virtue of their low cost in combination with their remarkably high strengths. This low cost is directly attributable to the low amount of alloying ingredients necessary to attain high strengths. As a matter of fact, high strengths can be obtained with alloying additions of about 0.13% consisting of about 0.05% beryllium and about 0.08% titanium.

Although the present invention has been described in conjunction with preferred embodiments, it is to be understood that modifications and variations may be resorted to without departing from the spirit and scope of the invention, as those skilled in the art will readily understand. For example, it is advantageous to use high-purity copper, e.g., oxygen-free copper, and high purity zinc particularly where high electrical conductivity is an important factor. Such modifications and variations are considered to be within the purview and scope of the invention and appended claims.

What is claimed is:

- An alloy consisting essentially of, by weight, about 0.05% to about 0.35% beryllium, about 0.08% to about 0.5% titanium, up to about 0.5% chromium, up to about 10% aluminum, about 10% to about 45% zinc with the sum of aluminum and zinc being about 10% to about 45%, less than about 0.1% lithium and the balance, apart from incidental elements, being copper in amounts of at least about 54.5%.
- An alloy consisting essentially of, by weight about

0.05% to about 0.1% beryllium, about 0.08% to about 0.2% titanium, up to about 0.1% chromium, up to about 7% aluminum, about 10% to about 45% zinc with the sum of aluminum and zinc being about 10% to about 45%, less than about 0.1% lithium and the balance essentially copper in amounts of at least about 54.5%.

3. An alloy consisting essentially of, by weight, about 0.05% to about 0.085% beryllium, about 0.08% to about 0.12% titanium, up to about 0.1% chromium, up to about 5% aluminum, about 10% to about 45% zinc with the sum of the aluminum present and zinc being about 10% to about 45%, less than about 0.1% lithium and the balance essentially copper in amounts of at least about 54.5%.

4. An alloy consisting essentially of, by weight, about 0.05% to about 0.085% beryllium, about 0.08% to about 0.12% titanium, about 0.015% to 0.02% chromium, up to about 5% aluminum, about 15% to about 40% zinc with the sum of the aluminum present and zinc being about 15% to about 40% and the balance, apart from incidental elements, being copper in amounts of at least about 60%.

5. A high-strength copper-zinc alloy having good conductivity consisting essentially of, by weight, about 0.05%

to about 0.35% beryllium, about 0.08% to about 0.5% titanium, up to about 0.5% chromium, about 10% to about 45% zinc with the balance, apart from incidental elements in amounts of less than about 0.3%, being copper in amounts of at least about 54.5%.

6. A high-strength copper-zinc alloy having good conductivity consisting essentially of, by weight, about 0.05% to about 0.085% beryllium, about 0.08% to about 0.12% titanium, up to about 0.1% chromium, about 15% to about 40% zinc with the balance, apart from incidental elements in amounts of less than about 0.1%, being copper in amounts of at least about 60%.

#### References Cited

##### UNITED STATES PATENTS

|           |        |        |       |            |
|-----------|--------|--------|-------|------------|
| 2,408,342 | 9/1946 | Rodda  | ----- | 75—157.5   |
| 3,166,410 | 1/1965 | Hanson | ----- | 75—157.5 X |

##### FOREIGN PATENTS

|         |         |                |
|---------|---------|----------------|
| 683,122 | 11/1952 | Great Britain. |
| 954,288 | 4/1964  | Great Britain. |
| 96,603  | 6/1960  | Norway.        |

CHARLES N. LOVELL, *Primary Examiner.*